

June 28, 1960

N. L. CARR

2,943,127

HYDROCARBON ISOMERIZATION PROCESS AND CATALYST TREATMENT

Filed Nov. 5, 1957



BY INVENTOR

NORMAN L. CARR

*Edward H. Lang*  
ATTORNEY

## HYDROCARBON ISOMERIZATION PROCESS AND CATALYST TREATMENT

Norman L. Carr, Crystal Lake, Ill., assignor to The Pure Oil Company, Chicago, Ill., a corporation of Ohio

Filed Nov. 5, 1957, Ser. No. 694,586

13 Claims. (Cl. 260—683.65)

This invention relates to the catalytic hydroisomerization of isomerizable, C<sub>5</sub>—C<sub>7</sub> hydrocarbons. It is more specifically directed to the upgrading of low-octane-number hydrocarbon feed stocks derived from crude petroleum oils.

In the processing of crude petroleum oils for the manufacture of high-octane gasolines, a variety of unit processes are employed in treating the distillate stocks to provide blending stocks which may be employed in the formulation of a finished gasoline-type motor fuel. The major constituent of a gasoline pool is the gasoline derived from the catalytic cracking of gas oils obtained from the distillation of the petroleum oil. Various schemes involving polymerization and alkylation are available for processing the available, normally gaseous, feed stocks. Generally, the C<sub>5</sub>+, virgin gasolines are catalytically hydroformed to cyclize and aromatize the constituents of the feed stock which response to this type of treatment. Although isomerization is one of the concomitant reactions in the hydroforming process, this is a competing equilibrium-type reaction. Accordingly, maximum efficiency is not obtained with respect to this particular reaction. Furthermore the hydroforming type of refining processes yields gasoline blending stocks which have a high research octane number, but they have high sensitivity because the improvement in motor octane value and research octane value is not effected at the same rate. Fuels which are suitable for use in high-speed, high-output, spark-ignited internal combustion engines preferably have a relatively low sensitivity. One particular technique for reducing fuel sensitivity is to incorporate in the finished gasoline isomerized, straight-run components. Accordingly, it is desirable to employ an isomerization process in a refining scheme for the production of a finished, high-octane-number gasoline having low sensitivity. In general, the isomerizable feed stock is taken from a C<sub>5</sub>+, virgin gasoline stock and constitutes a straight-run or natural gasoline feed stock, having an ASTM boiling range of from about 90° F. to about 210° F., containing substantial amounts of isomerizable, straight-chain paraffinic hydrocarbons.

A number of liquid-phase isomerization processes employ a Friedel-Crafts-type catalyst, and vapor-phase isomerization processes using solid catalyst have been developed. The efficiency of these processes is considerably influenced by the type of catalyst employed.

Therefore, it is the primary object of this invention to provide a non-corrosive, highly selective, solid catalyst for the conversion of normal pentane, normal hexane and normal heptane or mixtures thereof to high-octane-number, branch-chain isomers at a high yield. Another object of this invention is to prepare an isomerization catalyst which is employed in the hydroisomerization of suitable isomerizable feed stocks at a temperature of about 600—750° F., a pressure of from about 180 to 1000 p.s.i., and a hydrogen/hydrocarbon mol ratio of about 0.5 to 4.5. It is another object of this invention to provide a hydroisomerization process for the upgrading of low-

boiling-point, petroleum-derived hydrocarbon feed stocks containing normal pentane, normal hexane and normal heptane to provide high-octane-number blending stocks which can be utilized in the formulation of high-octane-number gasolines having low sensitivity.

Figure 1 is a graphical presentation of the effect of the partial pressure of water in the processing hydrogen, and of the temperature of the processing step on the water content of the catalyst.

10 Figure 2 illustrates the effect of including selected amounts of water in the hydrogen conditioning gas employed in the process of this invention for specific SiO<sub>2</sub>—Al<sub>2</sub>O<sub>3</sub> catalyst compositions prepared by incorporating the promoter in the "green" catalyst as NiMoO<sub>4</sub>, and subsequently activating.

15 Investigators of the isomerization process catalyzed by a solid type of catalyst have found that a catalyst composite prepared by incorporating small amounts of a hydrogenation agent on an acidic oxide catalyst support, 20 said support composited to evince acidic properties and hydrocarbon cracking activity, are active and selective for the hydroisomerization of C<sub>5</sub>—C<sub>7</sub> isomerizable hydrocarbons. A variety of acidic oxides of this nature which can be employed in the preparation of such catalysts are 25 the known hydrocarbon cracking catalysts. These include but are not limited to silica-alumina, silica-zirconia, silica-titania, silica-boria, alumina-zirconia, alumina-beryllia, alumina-boria, silica-chromia, boria-titania, silica-alumina-zirconia, silica-alumina-beryllia, acid-treated clays, etc. The oxides employed in forming the base can be either in chemical or physical combination.

30 It has been found according to this invention that selected promoters, when incorporated in the acidic oxide catalyst base, are receptive to a catalyst treatment technique which enhances the hydroisomerization efficiency of the composite catalyst. Heat-stable promoters which are used in the preparation of promoted, acidic oxide, hydroisomerization catalysts include group VIII metals of the iron series; group VIII metal of the iron series salts of the oxy-acids of tungsten, and molybdenum; and the oxides of molybdenum and tungsten. For example, iron, nickel, or cobalt; iron, nickel, or cobalt molybdate or tungstate; or molybdenum or tungsten oxide.

35 In the preparation of catalysts of this nature, the composite is activated in the final step of the catalyst preparation in the presence of hydrogen, or subjected to a hydrogen treatment prior to use, in order to reduce the reducible metal ions in the catalyst composition to substantially the lowest state of valency under the conditions of reduction. A variety of methods have been devised and 40 are described in the prior art for preparing these catalysts. For example, catalyst comprising silica-alumina and group VIII metals can be prepared impregnating the silica-alumina carrier with a solution of a soluble group VIII metal salt, such as the acetate, nitrate, or complex group 45 VIII metal ammonium compound, or the molten salt may be employed in impregnating the silica-alumina. The group VIII metal is then produced by decomposing and reducing the compound with a reducing gas, such as hydrogen. Another technique involves the mixing of a solution of a group VIII metal salt with the silica-alumina carrier. A group VIII metal hydroxide or carbonate is then precipitated to effect the impregnation of the silica-alumina. The resultant mixture is filtered, and the impregnated silica-alumina is washed free of soluble salts and dried, after which the group VIII metal is produced by decomposition and reduction of the hydroxide or carbonate. In certain instances it may be preferred to 50 heat the impregnated group VIII metal compound in a suitable oxidizing atmosphere prior to reduction to the group VIII metal. A more recent technique for the 55

preparation of a silica-alumina carrier having incorporated therein a highly active, finely divided catalyst involves impregnating silica-alumina with solution of a complex group VIII metal ammonium salt, and thereafter contacting the impregnated silica-alumina with carbon dioxide to produce the carbonate. The impregnated carrier is then dried and calcined at a temperature at which the carbonate will decompose to form the oxide, after which the oxide is subjected to reduction to form the metallic catalyst. It is essential in preparing catalysts of this nature, wherein an ammonium compound is employed in the catalyst preparation, that reducing conditions of time and temperatures sufficient to effect the substantially complete removal of ammonium ions from the catalyst be utilized in order to avoid adversely affecting catalyst activity. In the event that group VIII metal of the iron series salts of oxyacids of molybdenum, or tungsten, or the oxides of molybdenum or tungsten are employed in preparing the composite catalyst, the catalysts are treated at elevated temperatures with a suitable free hydrogen-containing or -producing agent in order to reduce the reducible metal ions to substantially the lowest valency state obtainable at the reducing conditions employed.

The mixed oxide support can be prepared by separately mixing prepared proportions of refractory oxides which, when composited, will evince the necessary acidic characteristics and also have hydrocarbon cracking activity. In addition, these catalyst constituents can be prepared by conventional coprecipitation techniques. In other words, in preparing the acidic oxides-hydrogenation agent composite for use in carrying out the instant invention, any conventional catalyst synthesis can be utilized wherein the finishing step involves exposing the catalyst composition to a hydrogen atmosphere in order to effect the reduction of the reducible constituents of the catalyst composition to the lowest state of valency obtainable at the conditions of reduction.

It is known that special catalyst conditioning procedures are frequently employed in order to insure maximum catalytic activity. In accordance with this invention, it has been found that the promoted, acidic oxide composite, hydroisomerization catalysts employed in this invention can be improved with regard to yield, selectivity and stability by incorporating in a hydrogen-rich, treating-gas stream, employed in the ultimate step in the catalyst preparation and/or treatment, a partial pressure of water vapor and contacting the catalyst at an elevated temperature for a time sufficient to permit the interaction of water and the catalyst to reach equilibrium at the treating conditions employed. The partial pressure of the water vapor in the oxidizing and/or reducing gaseous stream depends upon the temperature at which the water equilibration is carried out. The selectivity is improved by treatment with water vapor at temperatures of not less than about 700° F.; however, the desirable range of partial pressure of water vapor is shifted to lower values as temperature is lowered. The role of the interaction between the catalyst and the water vapor, which produces the improved selectivity, decreases somewhat as the temperature is lowered to the 700° F. level. Consequently, although temperatures as low as about 700° F. can be used, if the rates at which equilibrium is reached are too slow, the water-equilibration is impractical and uneconomic.

In carrying out the catalyst treatment technique which is the subject matter of this invention, in one embodiment, a "green" catalyst is prepared in any suitable manner, such as outlined above. Thereafter the "green" catalyst is activated by employing a conventional oxidation-reduction cycle, or a simple reduction. In order to effectuate the objectives of this invention, the reducing gases which are utilized in this activation step are humidified in order to incorporate a suitable amount of water vapor in the gaseous treating stream.

To effect the evaporation of water into the processing gases, viz., reducing gaseous streams, for the purpose of humidifying the gases, conventional techniques can be used. To add sufficient amounts of water to provide the desired partial pressure, the humidity of the gas stream can be employed as the criterion if desired because this property is related to the partial pressure of the water being carried. If

5  $p$ =partial pressure (absolute units),

10  $P$ =total pressure of the gas-water mixture (absolute units),

$M_w$ =molecular weight of the water=18, and

$M_g$ =molecular weight of the gas, then

$$15 \text{ Humidity (lb. water/lb. dry gas)} = \left( \frac{p}{P-p} \right) \left( \frac{18}{M_g} \right)$$

In addition, water partial pressure can also be calculated from the wet-bulb depression of the processing gas resulting from its humidification or dehumidification (see Unit Operations, Brown et al., Wiley, 1950, chap. 37). Humidification of the processing gases preferably is carried out using an indirect system in which the water is sprayed into the processing gas before it contacts the catalysts being water-equilibrated. To determine the proper humidity conditions, although the processing streams employed will not be air, results within the range of engineering accuracy will be obtained employing proper units on humidity charts for air-water systems. Of course, if the psychrometric properties of the processing gas system actually to be employed are available, these should be used.

20 30 In carrying out the instant invention, although other humidification procedures can be used, it is preferred that an indirect humidification system be employed, such as a packed tower wherein water and the processing gas are countercurrently contacted, under conditions such that the gas is saturated with water at the selected conditions of temperature and pressure. At dynamic equilibrium conditions, the vapor pressure of the water will be equal to the partial pressure of water in the processing-gas effluent from the humidifier. Although this assumes ideal gas conditions, analysis of the effluent processing gas corroborates the accuracy of this technique. In general, the humidification will be carried out at pressures within the range of 0 to 50 p.s.i.g. and at a temperature selected to effect the desired humidification, generally within the range of about 50 to 100° F.

35 40 45 50 The humidified processing gas is then heated to the selected processing temperature and the catalyst composition treated until not only the desired functional effect of the processing step, viz., reduction of the reducible constituents of the catalyst composition is effected, but water equilibration of the catalyst composition by the humidified processing stream is accomplished. This latter condition is indicated by the absence of any substantial difference between the water partial pressure in the processing gas introduced into the catalyst bed and the effluent removed.

60 65 Because controlled humidification of the activation gases is an important aspect of the instant invention, it is necessary that the concentration of water in the activation streams be controlled within narrow ranges depending upon the activation temperature. Reference is made to Fig. 1 which shows a graphical presentation of various

70 75 temperatures which can be employed in activating the promoted acidic oxide composite hydroisomerization catalyst employed in this invention. It will be noted that a circumscribed area is provided on this graphical presentation. According to this invention, control of the partial pressure of water in the free-hydrogen-containing treating gases must be maintained within this area and correlated with a selected treating temperature to obtain maximum efficiency.

To illustrate the effectiveness of the instant invention,

a catalyst, a nickel, molybdenum oxide, silica-alumina catalyst composite, was prepared as follows:

An ammoniacal solution of para-molybdate was prepared by dissolving 32 grams of ammonium heptamolybdate



in 270 ml. of distilled water to a salt content of about 11% by weight. To this solution was added 20 cc. of concentrated ammonium hydroxide to provide an



ratio of about 0.075/1. An 18 weight percent solution of nickel nitrate was prepared by dissolving 58.7 grams of  $Ni(NO_3)_2 \cdot 6H_2O$  in 270 ml. of water, and the molybdenum- and nickel-containing solutions were separately heated to about 176° F. and admixed. To this mixture was added 360 grams of silica-alumina, sufficient to yield a composition containing 10% of nickel molybdate. The composition of the commercially prepared, silica-alumina, hydrocarbon cracking catalyst<sup>1</sup> was:

| Component: | Wt. percent |
|------------|-------------|
| $Al_2O_3$  | 23.13       |
| $Na_2O$    | 0.02        |
| Fe         | 0.02        |
| $SO_4$     | 0.25        |
| $SiO_2$    | 76.59       |

The resulting slurry was mixed for one hour at 176° F., and then was filtered, washed with water, pelleted to provide  $\frac{1}{8}$ " pellets, and dried for 16 hours in an oven at 230° F. to provide a "green" composite containing 10%  $NiMoO_4$  on the silica-alumina support.

To activate the catalyst, employing a conventional catalyst preparation, 170 ml. of "green" catalyst "A" was inserted in a reactor and heated rapidly to 400° F. with 10 s.c.f.h. of hydrogen flowing through the reactor. The temperature of the catalyst was raised, at a rate of 100° F. per hour, to 975° F. employing a hydrogen rate of 10 s.c.f.h. This hydrogen rate and temperature was maintained for one hour after which the hydrogen rate was reduced to 4 s.c.f.h. and held for 6 hours at 975°, until no ammonia was detected in the off gas. The catalyst was then cooled to run temperature and employed in the n-pentane isomerization run defined in Table I.

Another batch of 150 ml. of "green" catalyst ("B"), similarly prepared, was disposed in a reactor. This catalyst was decomposed as was catalyst "A," except that the time at 975° F. was 29 hours. The temperature then was lowered to 825° F. at which level the catalyst was equilibrated with hydrogen containing moisture, at a level of 22 mm. (mercury) partial pressure, for 50 hours. The conditions were then changed to those of the defined run. The result is noted under column heading (1) in Table I. Another example with the same catalyst, but treated at different conditions with moisture in the hydrogen, is given under heading (2), Table I.

These catalysts were disposed in a reactor under suitable reaction conditions, and a feed stock consisting essentially of normal pentane was introduced into the reaction system and processed under isomerization conditions. As mentioned, the results of these runs are tabulated in Table I. The effectiveness of the instant invention is readily seen when the conversion, yield, and selectivity results for the preconditioned catalysts are compared with the results from the virgin or untreated catalyst. In addition to lower yield results, catalyst "A" produced excessive hydrocracking.

The effect of employing water partial pressures outside the critical range is illustrated by Figure 2.

Although the advantages which are obtained by the

6  
TABLE I  
Processing conditions

|                       |     |
|-----------------------|-----|
| Temperature, °F.      | 700 |
| Pressure, p.s.i.g.    | 500 |
| $H_2/n-C_5$ mol ratio | 1.0 |
| LVHSV <sup>1</sup>    | 3.3 |

| 10 | Conventionally Prepared Catalyst "A"   | Water Equilibrated Catalyst "B" |             |
|----|----------------------------------------|---------------------------------|-------------|
|    |                                        | (1)                             | (2)         |
| 15 | n-Pentane conversion.....              | 51                              | 41.0 41.7   |
|    | 1-Pentene yield.....                   | 35                              | 37.8 39.2   |
|    | Selectivity.....                       | 68                              | 92.3 93.9   |
| 20 | Reaction Effluent, Wt. Percent Charge: |                                 |             |
|    | Methane.....                           |                                 | 0.58 0.52   |
|    | Ethane.....                            |                                 | 0.12 0.29   |
|    | Propane.....                           |                                 | 0.30 0.55   |
|    | Butane.....                            |                                 | 1.83 1.28   |
|    | Isopentane.....                        | 35.6                            | 38.73 40.05 |
|    | n-Pentane.....                         | 46.9                            | 55.96 55.23 |
|    | Cyclopentane + hexane.....             | 1.6                             | 2.3 2.13    |

<sup>1</sup> Liquid volume hourly space velocity.

<sup>2</sup> This catalyst was actually too "hot" to operate satisfactorily in an isothermal reactor; it would be impossible to operate adiabatically. This is because of the high exotherm nature of the hydrocracking reaction.

instant invention are illustrated by the data in Table I, which are with a virgin catalyst of high activity and selectivity, the instant invention also has application in the hydrogen treatment of a regenerated, spent catalyst to provide a revivified catalyst having a high selectivity and activity. This phase of the instant invention is carried out as a supplementary step in a conventional oxidation-reduction cycle, regeneration process wherein a spent, promoted, acidic oxide, hydroisomerization catalyst is oxidized at a temperature within the range of about 850° to 950° F. In the oxidizing step a suitable, free-oxygen containing gas, e.g., air, is employed. If desired, the temperature of the catalyst bed, after the burning has ceased, can be raised to not higher than about 950°-1000° F. This high temperature is to be initially avoided during the oxidation step because the resulting sintering causes a substantial reduction in activity and surface area. The oxidized catalyst is thereafter reduced at a temperature of about 950°-1000° F. in the presence of a free-hydrogen-containing gas. In this step the hydrogen-containing gas is introduced at a suitable rate for about 10 to 30 hours to effect the reduction of the reducible constituents of this catalyst.

If the water-equilibration aspects of this invention are employed in the preconditioning of a catalyst composition which has been previously activated by treatment with a free-hydrogen-containing reducing gas, another important factor which affects the level of activity is the water content of the hydrogen employed in this reducing step prior to water-equilibration. This condition has been termed "catalyst dryness," and is defined as the moisture level in the hydrogen employed in the reduction phase of the activation or regeneration at catalyst conditions of about 975° F. for a time sufficient to produce a catalyst in equilibrium with the applied moisture. Generally, this requires treating the catalyst with a free-hydrogen-containing gas containing water for 15-30 hours to effect the concomitant reduction of the reducible constituents of the catalyst and the desired equilibration. In Table II are shown data which illustrate that the catalyst dryness plays an important part in activity, and that the catalyst should be treated with dry hydrogen in the reduction phase of the activation or regeneration cycle for best results.

It is also desirable in employing the process of this invention in conjunction with the regeneration of the selected, promoted, acidic oxide, hydroisomerization catalyst employed in this invention to avoid the use of an intermediate, vacuum-purging step in the oxidation-re-

7  
TABLE II

| Catalyst dryness in terms of degree of water in equilibrating gas, mm. Hg. | Percent iC <sub>5</sub> Yield at Constant Operating Conditions |
|----------------------------------------------------------------------------|----------------------------------------------------------------|
| 0-5 (dry)                                                                  | 38                                                             |
| 15                                                                         | 28.8                                                           |
| 22                                                                         | 22.7                                                           |

generation cycle because this step can lead to substantial decrease in activity when there is considerable sulfur added to the catalyst during processing.

It is also preferred to utilize a two-level temperature treatment in the water-equilibration treatment of this invention. The higher temperature is generally within the range of 925° to 975° F., and the lower temperature is a temperature above the temperature used in the hydro-isomerization process, viz., 700-850° F., but about 75° to 275° F. lower than the initial temperature. It has been found, for example, that two-level treatments employing temperatures of 975° and 800° F., and 975° and 700° F., respectively, provide an increase of 3.5 selectivity units with a concomitant butane production rate of one-half as compared with a one-level temperature treatment at the lower temperature.

Although the foregoing illustrative embodiments of this invention utilize a nickel-containing promoter incorporated in a silica-alumina hydrocarbon cracking catalyst base, it is to be understood that the instant invention is broadly directed to decreasing hydrocracking reaction rates by the water-equilibration of composite catalysts consisting essentially of a major portion of a refractory acidic oxide catalyst, composited to evince hydrocarbon cracking activity and acidic properties, and a minor portion of a promoter selected from the group consisting of group VIII metals of the iron series, e.g., Ni-SiO<sub>2</sub>-Al<sub>2</sub>O<sub>3</sub>; group VIII metal of the iron series salts of an oxyacid of tungsten or molybdenum, e.g., nickel molybdate-silica-alumina and nickel-tungstate-silica-zirconia; and the oxides of molybdenum or tungsten, e.g., tungsten oxide-silica-alumina, molybdenum oxide-silica-zirconia, especially for use in the isomerization of C<sub>5</sub>-C<sub>7</sub> isomerizable hydrocarbons. In the promoter, the metal ions exist in substantially their lowest state of valency attainable at the reducing conditions utilized in the catalyst preparation.

The catalyst composition will consist essentially of the acidic oxide catalyst support having incorporated therein 0.5 to 8% by weight of a single, selected promoter. To facilitate a determination of the amount of promoter to be employed, and because of the inability to define the promoter constituents in their reduced state with precision, it is preferred that these amounts be based upon the proportion of promoter incorporated in the catalyst composite prior to activation, whereby the valency state of the reducible ions in the promoter may have been lowered, and/or the catalyst water equilibrated. Preferred supports are the silica-alumina hydrocarbon cracking catalysts having silica contents within the range of about 50-95 wt. percent; however, other acidic oxides compositions can be used. Preferred promoters used to initially prepare the catalyst, and which are subjected to further treatment to effect their reduction, are nickel-containing materials, for example, metallic nickel, nickel molybdate, other combinations of nickel and molybdenum oxides, and similar materials. As discussed above, the water-equilibration is carried out by incorporating a small amount of water in the hydrogen treating agent employed in the conditioning step. The water is added to the reducing gases in small amounts depending upon treating temperature. The following represents in tabular form a summary of the partial pressure condition that should exist within the gas streams employed in the pre-conditioning step.

8

| Temperature°, F. | Water Partial Pressure, mm. Hg abs. |             |
|------------------|-------------------------------------|-------------|
|                  | Lower Limit                         | Upper Limit |
| 5                |                                     |             |
| 700              | 5                                   | 25          |
| 825              | 10                                  | 40          |
| 975              | 15                                  | 100         |

10 The water equilibration step of this invention has application in improving the activity and selectivity of the above-mentioned promoted acidic oxides in a variety of catalyst preparations and techniques. In general, the water equilibration is the final step in the catalyst treatment wherein a humidified, free-hydrogen-rich gas having a water partial pressure, depending upon the treating temperature, within the range of 5-100 mm. of mercury absolute, and preferably 10-30 mm., is employed to effect the desired improvement in catalyst properties. The humidified hydrogen is introduced at a rate and for a time sufficient to bring the catalyst composition being treated into equilibrium with the treating gas, and, depending upon the state of the catalyst composition being treated, to effect the reduction of the reducible ions of the catalyst composition to the lowest state of valency attainable at the treating conditions. In general, the humidified hydrogen is introduced at a linear rate within the range of 10 to 100 feet per minute for about 2-20 hours employing a temperature within the range of about 700°-975° F.

15 Accordingly, the water-equilibration, catalyst treating step of this invention can be used as a concomitant activation and conditioning step in the activation of a "green" catalyst; as a supplementary hydrogen treatment in the conditioning of an active catalyst wherein the selected promoting agents are reduced and are at the lowest state of valency obtainable under the reduction conditions employed in the catalyst activation; in the enhancement in efficiency of a regenerated, spent catalyst which has been 20 revivified by means of a sequential oxidation-reduction cycle; or in various other catalyst preparations, which, in view of the foregoing discussion, will be apparent to those skilled in this art.

25 Although the instant invention has application as a unit process for the isomerization of suitable hydrocarbon feed stocks, it is advantageously employed in conjunction with a reforming or hydroforming operation wherein selected hydrocarbon feed stocks are transformed to high-octane-number gasoline-blending stocks. In carrying out the isomerization phase of this invention, the following 30 operating conditions are employed.

| Operating Conditions           | Range             | Preferred Range |
|--------------------------------|-------------------|-----------------|
| Temperature, °F.               | 600-750           | 650-700         |
| Pressure, p.s.i.a.             | Atmospheric-1,000 | 180-1,000       |
| Hydrogen/hydrocarbon mol ratio | 0.5-4.5           | 0.5-3.4         |

35 40 45 50 55 60 65 70 75 It is preferred that this combination be employed in order to effect substantial improvements in the yield-octane number relationship of the product obtained by the processing of a full-boiling-range, virgin naphtha in an integrated, isomerization-reforming process.

75 Another important aspect of the instant invention is the use of the so-called "split-stream" treatment of feed stocks in order to more advantageously process the respective constituents of the feed stocks. In other words, in employing the instant invention to effect maximum efficiency in the processing of a feed stock containing an admixture consisting predominantly of normal pentane, normal hexane, and normal heptane, it is preferred that each constituent be separately treated in reaction systems designed and operated under conditions especially adapta-

ble for obtaining maximum effectiveness. Reaction systems may be designed for treating a combination n-C<sub>5</sub>-n-C<sub>6</sub> stream and a n-C<sub>7</sub> stream, the processing of each of the principal constituents separately, or the processing of a n-C<sub>6</sub> stream and the processing of a combination normal hexane, normal heptane stream. This, of course, requires prefractionation of the feed stock in order to provide satisfactory feed streams.

The instant invention is directed to the improvement of isomerization catalysts for use in the processing of n-C<sub>5</sub>-C<sub>7</sub>-containing feed stocks, either to effect their skeletal isomerization per se, or to prepare high-octane-number blending stocks used in the formulation of motor fuels especially adapted to high-output, high-speed, spark-ignited, internal combustion engines. Although the invention is illustrated with reference to specific catalyst compositions and specific operating conditions, it is obvious that modifications in the catalyst preparation and isomerization other than those specifically set forth above can be made by those skilled in the art.

Accordingly it is intended that the instant invention be limited only in the manner defined in the following claims.

I claim as my invention:

1. In a process for improving the selectivity, yield and stability of a hydroisomerization catalyst composite consisting essentially of a major portion of a refractory, acidic oxide catalyst support, containing 50-95% wt. silica, composited to evince acidic properties and hydrocarbon cracking activity, and a minor amount of at least one promoter selected from the group consisting of group VIII metals of the iron series, salts of group VIII metals of the iron series and oxyacids of molybdenum and tungsten, and oxides of tungsten and molybdenum, the ultimate step which comprises contacting said catalyst composite with a humidified, hydrogen-rich gas, having a partial pressure of water and a temperature within the shaded area of Fig. 1, for a time sufficient to permit the interaction between the water in said gas and the catalyst composite to reach equilibrium at the contacting conditions employed.

2. In a process for improving and selectivity, yield and stability of a hydroisomerization catalyst composite consisting essentially of a major portion of a refractory, acidic oxide catalyst support, containing 50-95% wt. silica, composited to evince acidic properties and hydrocracking activity, and a minor amount of at least one promoter selected from the group consisting of group VIII metals of the iron series, salts of group VIII metals of the iron series and oxyacids of molybdenum, and tungsten, and oxides of tungsten and molybdenum, the ultimate step which comprises contacting said catalyst composite with a humidified, hydrogen-rich gas, having a partial pressure of water and a temperature within the shaded area in Fig. 1, for a time sufficient to permit the interaction between the water in said gas and the catalyst composite to reach equilibrium and to effect the reduction of the reducible metal ions of the promoter to their lowest state of valency under the hydrogen treatment conditions employed.

3. A process for improving the selectivity, yield and stability of a hydroisomerization catalyst composite consisting essentially of a major portion of a refractory, acidic oxide catalyst support, containing 50-95% wt. silica, composited to evince acidic properties and hydrocarbon cracking activity, and a minor amount of at least one promoter selected from the group consisting of group VIII metals of the iron series, salts of group VIII metals of the iron series and oxyacids of molybdenum and tungsten, and oxides of tungsten and molybdenum, which comprises preparing a "green" catalyst composite consisting of a composite of a major portion of said acidic oxide catalyst support and a small amount of said promoter, and thereafter activating and conditioning said catalyst by contacting said "green" catalyst with a hy-

drogen-rich reducing gas, having a water partial pressure and a temperature within the shaded area of Fig. 1, for a time sufficient to effect the reduction of the reducible metal ion constituents of the promoter to their lowest state of valency under the reducing conditions employed and to permit the interaction between the water in said gas and the catalyst composite to reach equilibrium at the contacting conditions employed.

4. In a process for improving the selectivity, yield and stability of an active hydroisomerization catalyst prepared by the hydrogen activation of a composite consisting essentially of a major portion of a refractory, acidic oxide catalyst support, containing 50-95% wt. silica, composited to evince acidic properties and hydrocarbon cracking activity, and a minor amount of at least one promoter selected from the group consisting of group VIII metals of the iron series, salts of group VIII metals of the iron series and oxyacids of molybdenum and tungsten, and oxides of tungsten and molybdenum, the 15 reducible metal ions of said promoter being at their 20 lowest state of valency obtainable by said hydrogen activation, the ultimate step which comprises contacting said catalyst composite with a humidified, hydrogen-rich gas, having a partial pressure of water and a temperature within the shaded area of Fig. 1, for a time sufficient to 25 permit the interaction between the water in said gas and the catalyst composite to reach equilibrium at the contacting conditions employed.

5. In a process for improving the selectivity, yield and stability of a regenerated, hydroisomerization catalyst composite consisting essentially of a major portion of a refractory acidic oxide catalyst support, containing 50-95% wt. silica, composited to evince acidic properties and hydrocarbon cracking activity, and a minor amount of at least one promoter selected from the group consisting of group VIII metals of the iron series, salts of group VIII metals of the iron series and oxyacids of molybdenum and tungsten, and tungsten oxide and molybdenum oxide, said hydroisomerization catalyst having 30 been regenerated by a sequential oxidation-reduction cycle, the ultimate step which comprises contacting said catalyst composite with a humidified, hydrogen-rich gas, having a partial pressure of water and a temperature within the shaded area in Fig. 1, for a time sufficient to 35 permit the interaction between the water in said gas and the catalyst composition to reach equilibrium at the contacting conditions employed.

6. A process for improving the selectivity, yield and stability of a hydroisomerization catalyst composite consisting essentially of a major portion of a refractory, acidic oxide catalyst support, containing 50-95% wt. silica, composited to evince acidic properties and hydrocarbon cracking activity, and 0.5 to 8%, by weight, based on the amount initially incorporated in said composite, 50 of a promoter selected from the group consisting of group VIII metals of the iron series, salts of group VIII metals of the iron series and oxyacids of molybdenum and tungsten, and oxides of tungsten and molybdenum, the ultimate step which comprises contacting said catalyst composite with a humidified, hydrogen-rich gas, having a partial pressure of water and a temperature within the shaded area of Fig. 1, for a time sufficient to 55 permit the interaction between the water in said gas and the catalyst composition to reach equilibrium at the contacting conditions employed.

7. In a process in accordance with claim 6 in which said hydroisomerization catalyst is a nickel molybdate-silica-alumina composite.

8. In a process for improving the selectivity, yield and stability of a hydroisomerization catalyst composite consisting essentially of a major portion of a refractory, acidic oxide catalyst support, containing 50-95% wt. silica, composited to evince acidic properties and hydrocarbon cracking activity, and a minor amount of at least 70 one promoter selected from the group consisting of group 75

VIII metals of the iron series, salts of group VIII metals of the iron series salt and oxyacids of molybdenum and tungsten, and oxides of molybdenum and tungsten, the ultimate step which comprises contacting said catalyst composite with a humidified, hydrogen-rich gas, having a partial pressure of water within the shaded area of Fig. 1, for a time sufficient to permit the interaction between the water in said gas and the catalyst composite to reach equilibrium, at the contacting conditions employed said contacting being carried out at a first elevated temperature within the shaded area of Fig. 1 and thereafter completing said contacting at a second elevated temperature which is lower than said first elevated temperature but is not less than the reaction temperature employed in the hydroisomerization process utilizing said hydroisomerization catalysts.

9. A process in accordance with claim 8 in which said first elevated temperature is 975° F., and said second elevated temperature is within the range of 700-800° F.

10. In a process for improving the selectivity, yield, and stability of a "green" hydroisomerization catalyst composite, consisting essentially of a major portion of a 50-95% wt. silica/50-5% wt. alumina hydrocarbon cracking catalyst and a minor portion of a nickel molybdate, the ultimate step which comprises contacting said catalyst composite with a humidified hydrogen-rich gas, having a partial pressure of water of 22 mm. of Hg, for a time sufficient to permit the interaction between the water and said gas and the catalyst composition to reach equilibrium, at the contacting conditions employed said contacting being carried out initially at a temperature of 975° F. and thereafter at a temperature within the range of 700°-800° F.

11. A hydroisomerization process which comprises contacting an isomerizable hydrocarbon having 5-7 carbon atoms per molecule in the presence of a hydroisomerization catalyst at a temperature within the range of

600°-750° F., a pressure in the range of 180-1000 p.s.i.g., and a hydrogen/hydrocarbon mol ratio within the range of 0.5-4.5, said hydroisomerization catalyst having been prepared by a process including the step of ultimately 5 contacting the catalyst consisting essentially of a major portion of a refractory, acidic oxide catalyst support, containing 50-95% wt. silica, composited to evince acidic properties and hydrocarbon cracking activity, and a minor amount of at least one promoter selected from the group 10 consisting of group VIII metals of the iron series, salts of group VIII metals of the iron series salt and oxyacids of molybdenum and tungsten, and oxides of tungsten and molybdenum, with a hydrogen-rich gas containing water 15 at a partial pressure and at a temperature within the shaded area in Fig. 1 for a time sufficient to permit the interaction between the water in said gas and the catalyst composition to reach equilibrium.

12. A process in accordance with claim 1 in which the isomerization catalyst comprises nickel molybdate supported on a 50-95% wt. silica/50-5% wt. alumina hydrocarbon cracking catalyst.

13. A process in accordance with claim 11 in which the isomerization catalyst comprises nickel molybdate supported on a 50-95% wt. silica/50-5% wt. alumina hydrocarbon cracking catalyst.

#### References Cited in the file of this patent

#### UNITED STATES PATENTS

|    |           |                        |                |
|----|-----------|------------------------|----------------|
| 30 | 2,292,570 | Klemm et al. -----     | Aug. 11, 1942  |
|    | 2,414,585 | Eggersten et al. ----- | Jan. 21, 1947  |
|    | 2,424,636 | Smith -----            | July 29, 1947  |
|    | 2,437,487 | Teter -----            | Mar. 9, 1948   |
|    | 2,438,584 | Stewart -----          | Mar. 30, 1948  |
| 35 | 2,718,535 | McKinley et al. -----  | Sept. 20, 1955 |
|    | 2,805,269 | Carter et al. -----    | Sept. 3, 1957  |
|    | 2,864,875 | McKinley et al. -----  | Dec. 16, 1958  |

UNITED STATES PATENT OFFICE  
CERTIFICATE OF CORRECTION

Patent No. 2,943,127

June 28, 1960

Norman L. Carr

It is hereby certified that error appears in the printed specification of the above numbered patent requiring correction and that the said Letters Patent should read as corrected below.

Column 1, line 32, for "response" read -- respond --; column 9, line 42, for "and" read -- the --; line 71, for "catalysyt" read -- catalyst --; column 10, line 35, for "gruop" read -- group --.

Signed and sealed this 20th day of December 1960.

(SEAL)

Attest:

KARL H. AXLINE

Attesting Officer

ROBERT C. WATSON  
Commissioner of Patents